

# UNITED STATES PATENT OFFICE.

ADOLF VOIGT, OF GIessen, GERMANY.

## EXPLOSIVE.

1,095,302.

Specification of Letters Patent.

Patented May 5, 1914.

No Drawing. Application filed March 29, 1911, Serial No. 617,714. Renewed March 21, 1914. Serial No. 826,440.

*To all whom it may concern:*

Be it known that I, ADOLF VOIGT, a subject of the German Emperor, residing at Giessen, Germany, have invented a new and useful Explosive; and I do hereby declare the following to be a full, clear, and exact description of the same.

While picric acid, as well as the salts of the same, and the corresponding cresol derivatives have frequently been used for explosive purposes, such use has, in recent years, shown a considerable decrease, owing to the high and increasing cost of the material, as compared with other explosives, and to the fact that the mentioned salts are highly sensitive to shock and to friction.

I have ascertained by experiments, that the mononitro and binitro derivatives of phenol, as well as of cresol, or the salts of the sulfo acids of the same, are not subject to the disadvantages mentioned, and have succeeded in producing explosives containing said ingredients intimately mixed with others. I have also ascertained that while the lower nitration products do not, alone, constitute explosives, yet that the addition thereto of oxygen carriers converts them into easily ignitable and extremely effective explosives. A combination for instance, of 25% sodium mononitro-phenolate and 75% sodium nitrate produces a mixture which is easily detonated and possesses the blasting force of black powder, and it is possible to treble the explosive force by the addition of potassium perchlorate. These mixtures, furthermore, are highly insensitive to blow and friction and do not ignite fire damp. The corresponding salts of sulfo acids show even better behavior. These offer the advantage that, they mix more freely with the nitrates, because they can be kept dry more easily than the technically pure mononitro phenol or cresol salts, and they furthermore increase the safety against the ignition of fire damp gases. This is especially true

in the case of ammonium salts of the nitro-phenol or nitro-cresol sulfo acids.

The preparation is carried on in such a manner that the nitro compounds are either intimately mixed with the nitrates and perchlorates, or they are together dissolved in water and evaporated, under stirring, until a granular crystalline substance is obtained. By this latter means a product of higher specific gravity is obtained.

The following proportions of mixture have proven especially suitable, depending upon the purposes for which same are to be used: (1) 25% sodium mononitrophenolate, or sodium nitro cresol sulfonate. 65% sodium or potassium nitrate. 10% potassium perchlorate or chlorate. (2) 25% sodium mononitrophenolate, or sodium nitro cresol sulfonate. 50% sodium or potassium nitrate. 25% potassium perchlorate or chlorate. (3) 22.5% sodium mononitrophenolate, or sodium nitro cresol sulfonate. 45% sodium or potassium nitrate. 22.5% potassium perchlorate or chlorate. 10% ammonium nitrate. (4) 25% sodium mononitrophenolate, or sodium nitro cresol sulfonate. 65% sodium or potassium nitrate. 10% trinitrotoluol. The mixtures which are detonated either by means of a fuse alone or by means of a detonator, can be varied according to the purposes for which they are to be used.

What I claim is:

An explosive compound comprising an intimate mixture of sodium nitro-cresol sulfonate, sodium nitrate and potassium perchlorate.

In testimony whereof, I have signed my name to this specification in the presence of two subscribing witnesses.

ADOLF VOIGT.

Witnesses:

ALBERT VOGELSSBERGER,  
JEAN GRUND.